

# United States Patent

[19]

Gray et al.

[11] 3,770,517

[45] Nov. 6, 1973

[54] **METHOD OF PRODUCING  
SUBSTANTIALLY NON-ORIENTED SILICON  
STEEL STRIP BY THREE-STAGE COLD  
ROLLING**

[75] Inventors: **Thomas H. Gray, Pittsburgh; Jack P. Martin, Lower Burrell, both of Pa.**

[73] Assignee: **Allegheny Ludlum Industries, Inc., Pittsburgh, Pa.**

[22] Filed: **Mar. 6, 1972**

[21] Appl. No.: **232,212**

## Related U.S. Application Data

[63] Continuation-in-part of Ser. No. 68,790, Sept. 1, 1970, abandoned.

[52] U.S. Cl. .... **148/111, 148/110, 148/112,**  
148/31.55

[51] Int. Cl. .... **H01f 1/04**

[58] Field of Search..... **148/111, 110, 112,**  
148/31.55, 120, 121

[56]

## References Cited

### UNITED STATES PATENTS

|           |         |                     |         |
|-----------|---------|---------------------|---------|
| 2,867,557 | 1/1959  | Crede et al. ....   | 148/111 |
| 3,513,039 | 5/1970  | Ganz. ....          | 148/111 |
| 2,992,952 | 7/1961  | Assmus et al. ....  | 148/111 |
| 2,067,036 | 1/1937  | Wimmer. ....        | 148/111 |
| 2,075,283 | 3/1937  | Heinzel et al. .... | 138/120 |
| 3,115,430 | 12/1963 | Jackson et al. .... | 148/111 |

Primary Examiner—L. Dewayne Rutledge

Assistant Examiner—W. R. Satterfield

Attorney—Vincent G. Gioia et al.

[57]

## ABSTRACT

Described is a method of producing substantially non-oriented silicon steel by a three-stage cold rolling process wherein the silicon steel is temper rolled in the third or last rolling stage after normalizing to effect a reduction in gauge of about 2 to 12 percent, followed by annealing at a temperature no greater than 1,700° F for a time no longer than about 5 minutes.

5 Claims, No Drawings

**METHOD OF PRODUCING SUBSTANTIALLY  
NON-ORIENTED SILICON STEEL STRIP BY  
THREE-STAGE COLD ROLLING**

**CROSS REFERENCES TO RELATED  
APPLICATIONS**

This application is a continuation-in-part of now abandoned copending application Ser. No. 68,790 filed Sept. 1, 1970 and assigned to the assignee of the present application.

**BACKGROUND OF THE INVENTION**

Present commercial applications have made use of silicon steels of the so-called oriented and non-oriented crystallographic texture. Oriented silicon steel products are normally manufactured from steels with high silicon contents and non-oriented products are usually made of steels with relatively lower silicon contents. For some uses, such as generator and motor components, there is a need for a quality grade of steel within a minimum magnetic isotropy. A.I.S.I. requirements have been established for these applications in terms of maximum core loss limits for the materials used. In the fully processed form (i.e., annealed condition), the maximum core loss for A.I.S.I. M-19 transformer grade is 1.64 watts per pound at 15 KB. Semi-processed (i.e., unannealed material) has a maximum core loss requirement for A.I.S.I. M-19 grade of 1.68 watts per pound at 15 KB.

**SUMMARY OF THE INVENTION**

The present invention provides a method for producing substantially non-oriented silicon steel, which complies with the A.I.S.I. M-19 requirements, from relatively high silicon steels such as the following:

| General Range | Element    | Typical |
|---------------|------------|---------|
| 2.90-3.40     | Silicon    | 3.15    |
| Traces 0.06   | Carbon     | 0.028   |
| 0.03-0.10     | Manganese  | 0.065   |
| Up to 0.03    | Sulfur     | 0.020   |
| Up to 0.020   | Phosphorus | 0.008   |
| 0.05 max.     | Aluminum   | <0.01   |
| 0.030-0.90    | Copper     | 0.080   |
| Up to 0.2     | Nickel     | 0.050   |

Among the advantages of utilizing high silicon material in the production of non-oriented silicon steel is the ability to employ a single melting and production practice while avoiding the need to manufacture multiple compositions for different purposes. That is, the high silicon steel can be used for both the non-oriented and oriented types. Another advantage is that the process of the invention permits the use of excess quantities of high silicon material which may be produced in the mill and which, by practicing the invention, can be diverted to the production of non-oriented products.

Previous attempts to produce non-oriented products by using high silicon steels have generally been unsatisfactory because of the necessity for utilizing high temperature annealing treatments to develop properties. Such requirements impose undue burdens on fabricators in terms of equipment needs and cost.

**DESCRIPTION OF PREFERRED EMBODIMENT**

In carrying out the invention, silicon steel containing 2.90 to 3.40 percent by weight of silicon is temper rolled in a normalized condition to effect a controlled reduction. Following temper rolling, the steel is then stress relief annealed, preferably at a temperature less

than 1,700° F. A typical process for producing the normalized steel of the invention is as follows:

1. Heat ingot for a minimum of 5 hours at a temperature over 2,300° F, including 3 hours at not less than 2,400° F.
2. Roll on blooming mill to produce a slab having a thickness of 5 to 8 inches and a temperature not less than 2,250° F.
3. Reduce the slab to a thickness of three-fourths to 1 1/2 inches and maintain at a temperature not less than 2,000° F. Such reduction is at a fast rate and preferably accomplished in three passes on a single strand reversing mill.
4. Admit the reduced slab at a temperature not less than 2,000° F to the first stand of a six-stand finishing mill and effect a reduction in the strip to a thickness of about 0.060 to 0.10 inch at a speed to insure a temperature not less than 1,600° F at the front and back end of the strip.
5. Descale the hot rolled strip.
10. Where desired, box or open anneal the hot rolled strip at a temperature between 1,400° and 2,000° F, followed by a descaling treatment.
15. Cold roll the annealed strip in a first cold rolling step to a thickness of about 1.3 to 2.5 times the final thickness.
20. Open anneal the cold rolled strip at a temperature between 1,600° and 1,850° F.
25. Cold roll in a second cold rolling step to a thickness approximately 2 to 12 percent greater than the desired final thickness.
30. Open anneal the cold rolled strip to normalize the same, preferably in a decarburizing atmosphere as in a wet reducing gas at a temperature substantially between 1,400° and 1,550° F.
35. Temper roll the normalized product to effect a reduction of about 2 to 12 percent.
40. Stress relief anneal at a temperature less than 1,700° F in a non-oxidizing atmosphere for up to about 5 minutes at temperature.
45. As can be seen, the process of the invention involves a three-stage cold rolling process wherein the last cold rolling step comprises temper rolling and wherein the strip is normalized between the second rolling step and the temper rolling step. Temper rolling to effect a reduction of about 2 to 12 percent has been found to be necessary to adequately destroy the potential for secondary recrystallization while controlling the tendency for recrystallization to occur at lower temperatures.
50. That is to say, it has been found that at least about a 2 percent reduction in the temper rolling step, and preferably about at least a 4 percent reduction, is desirable to produce material of minimum directionality. On the other hand, if the steel is unduly worked due to a reduction in temper rolling greater than about 12 percent, the minimum temperature for primary recrystallization is reduced and it will be difficult to obtain a coarsened primary recrystallized structure of the type desired for the intended applications.
55. The stress relief anneal, set forth in step 12 above, is preferably carried out at less than 1,700° F in a non-oxidizing atmosphere such as hydrogen or a nitrogen-hydrogen mixture for up to about 5 minutes at temperature. At these low annealing temperatures, however, little sulfur is removed. When low sulfur products are desired, therefore, a low sulfur material (e.g., less than 0.01 percent) should be used.

The following examples illustrate various embodiments of the invention:

Example No. 1

Steel having ladle chemistry shown in Table I was processed as normal oriented silicon steel strip would through final normalizing, whereupon it was tempered 10 rolled 8 percent —giving gages as shown in Table II and annealed at 1,500° F in pure, dry hydrogen for 15 minutes in hot zone of mesh belt furnace (~ 4 minutes at temperature). Properties obtained on Epstein packs of strips 1.5 × 15.25 cm. are also given in Table II. All results are of 60 cycle tests.

TABLE I

| C    | Mn   | P    | S    | Si   | Cr   | Ni   | Al   | Cu  | Sn   |
|------|------|------|------|------|------|------|------|-----|------|
| .029 | .058 | .006 | .025 | 3.05 | .027 | .068 | .005 | .10 | .011 |

TABLE II

|                      | High Loss<br>End of Coil | Low Loss<br>End of Coil |
|----------------------|--------------------------|-------------------------|
| All Longitudinal     |                          |                         |
| WPP at 15 KB         | 1.38                     | 1.26                    |
| All Transverse       |                          |                         |
| WPP at 15 KB         | 1.95                     | 1.91                    |
| ½ Long. - ½ Trans.   |                          |                         |
| WPP at 15 KB         | 1.60                     | 1.52                    |
| Final Gage of Sample | .0125"                   | .0124"                  |

Example No. 2

Steel of the same ladle chemistry of Example No. 1, was processed in the same manner except for being given a 7 percent temper roll to gage shown in Table III followed by a 1,600° F anneal in pure dry hydrogen. Properties of the steel are also shown in that table.

TABLE III

|                      | High Loss<br>End of Coil | Low Loss<br>End of Coil | 40 |
|----------------------|--------------------------|-------------------------|----|
| All Longitudinal     |                          |                         |    |
| WPP at 15 KB         | 1.31                     | 1.17                    |    |
| All Transverse       |                          |                         |    |
| WPP at 15 KB         | 1.78                     | 1.89                    |    |
| ½ Long. - ½ Trans.   |                          |                         |    |
| WPP at 15 KB         | 1.53                     | 1.48                    |    |
| Final Gage of Sample | .0125"                   | .0123"                  | 45 |

Example No. 3

Steel having the ladle chemistry given in Table IV was processed as normal oriented silicon steel strip until after final normalizing whereupon the sample was rolled 7 percent to gage shown, then annealed at 1,600° F in an 80 percent nitrogen + 20 percent hydrogen atmosphere for the same time as Examples 1 and 2. Properties on Epstein samples are shown in Table V.

TABLE IV

| C    | Mn   | P    | S    | Si   | Cr   | Ni   | Al   | Cu  | Sn   |
|------|------|------|------|------|------|------|------|-----|------|
| .026 | .056 | .009 | .022 | 3.20 | .032 | .074 | .005 | .13 | .012 |

TABLE V

|                      | High Loss<br>End of Coil | Low Loss<br>End of Coil |
|----------------------|--------------------------|-------------------------|
| All Longitudinal     |                          |                         |
| WPP at 15 KB         | 1.46                     | 1.42                    |
| All Transverse       |                          |                         |
| WPP at 15 KB         | 1.95                     | 2.03                    |
| ½ Long. - ½ Trans.   |                          |                         |
| WPP at 15 KB         | 1.65                     | 1.64                    |
| Final Gage of Sample | .0125"                   | .0124"                  |

It is apparent from the foregoing examples that all of the materials processed in accordance with the teachings of the invention have a core loss below 1.64 watts per pound at 15 KB, the maximum core loss for an A.I.S.I. M-19 transformer grade.

Although the invention has been described in connection with certain specific embodiments, it will be readily apparent to those skilled in the art that various changes in method steps and composition can be made to suit requirements without departing from the spirit and scope of the invention.

We claim:

1. A method of producing substantially non-oriented silicon steel strip exhibiting a core loss below 1.64 watts per pound at 15 KB, and consisting essentially in percent by weight of 2.9 to 3.4 percent silicon, traces to 25 0.06 percent carbon, 0.03 to 0.1 percent manganese, up to 0.03 percent sulfur, up to 0.02 percent phosphorus, 0.03 to 0.9 percent copper, up to 0.2 percent nickel, and the balance essentially iron, which comprises the steps of:

heating an ingot of silicon steel at a temperature in excess of 2,300° F,  
hot rolling said steel,  
descaling the hot rolled steel,  
cold rolling the hot rolled steel in a first cold rolling process to a thickness of 1.3 to 2.5 times the final thickness of the product,  
annealing the cold rolled strip at a temperature between 1,600° and 1,850° F,

cold rolling the annealed cold rolled strip in a second cold rolling operation to a thickness which exceeds the final thickness of the product by about 2 to 12 percent,  
normalizing the cold rolled steel after the second cold rolling operation at a temperature between 1,400° and 1,550° F,

temper rolling the normalized steel to effect a reduction of about 2 to 12 percent to achieve the final thickness of the product, and

stress relief annealing the temper rolled steel at a temperature no greater than 1,700° F and for a time period no greater than 5 minutes.

2. The method of claim 1 wherein said steel is tempered to effect a 4 to 12 percent reduction.

3. The method of claim 1 wherein said steel is stress relief annealed in a non-oxidizing atmosphere.

4. The method of claim 3 wherein said steel is stress relief annealed in a hydrogen-containing atmosphere.

5. The method of claim 1 wherein said steel has less than 0.01 percent sulfur.

\* \* \* \* \*